

## UNITED STATES PATENT OFFICE

ROBERT E. WILSON, OF CHICAGO, ILLINOIS, ASSIGNOR TO STANDARD OIL COMPANY, OF WHITING, INDIANA, A CORPORATION OF INDIANA

## ANTIKNOCK COMPOUNDS

No Drawing.

Application filed November 8, 1924. Serial No. 748,721.

The present invention relates to improvements in anti-knock compounds intended to be added to fuels of the gasoline type to prevent detonation or knocking in internal-combustion engines.

Mixtures of this type are known which contain as their principal constituents tetraethyl lead and an ethylene bromide compound, such as ethylene dibromide or ethylene chlorobromide. These mixtures usually contain, in addition to these constituents, a diluent such as kerosene, a known mixture consisting of tetraethyl lead, 6 parts; ethylene dibromide, 4 parts; and kerosene, 5 parts.

The use of mixtures of this character has been found to be objectionable, particularly in winter weather and in the northern parts of the United States, by reason of their relatively high freezing points. A mixture of the character above set forth has a freezing point in the neighborhood of about 14° F., which causes great difficulties in its handling and dispensing at freezing temperatures and below.

It has now been found that this objectionable feature of mixtures such as that above described may be obviated by replacing a part or all of the ordinary diluent, such as kerosene, with a miscible diluent liquid having an internal pressure between 0.90 and 1.08 (relative to the internal pressure of naphthalene as one). Thus, I may employ, as the miscible diluent, xylene, solvent naphtha, chlorbenzene, nitrobenzene or the like. For example, if, in the mixture above set forth, one half of the kerosene is replaced by xylene or solvent naphtha, the freezing point of the mixture is reduced to about 5° F.; and if all of the kerosene is replaced by xylene or solvent naphtha, the freezing point is reduced to about -18° F. Substantial reductions in the freezing point of the mixture result from the use of chlorbenzene, nitrobenzene, and other diluent miscible liquids having internal pressures in the range above set forth.

The term freezing point, as used herein, indicates the temperature at which, on cooling, separation of crystals of the ethylene bromide compound appears.

I claim:

1. A concentrated anti-knock composition for addition in relatively small proportions to gasoline and like motor fuels comprising as its principal constituents tetraethyl lead, an ethylene compound containing halogen atoms at least one of which is a bromine atom, and an additional miscible diluent liquid having an internal pressure between 0.90 and 1.08. 55

2. A concentrated anti-knock composition for addition in relatively small proportions to gasoline and like motor fuels comprising as its principal constituents tetraethyl lead and an ethylene compound containing halogen atoms at least one of which is a bromine atom, 60 xylene.

3. A concentrated anti-knock composition for admixture in relatively small proportions with gasoline and like motor fuels comprising as its principal constituents tetraethyl lead, ethylene dibromide, and a diluent consisting of equal parts of kerosene and xylene. 70

4. A concentrated anti-knock composition for admixture in relatively small proportions with gasoline and like motor fuels comprising tetraethyl lead 6 parts, ethylene dibromide 4 parts, and 5 parts of a diluent consisting of equal parts of kerosene and solvent naphtha. 75

5. A concentrated anti-knock composition for addition in relatively small proportions to gasoline and like motor fuels, comprising as its principal constituents tetraethyl lead, an ethylene compound containing halogen atoms at least one of which is a bromine atom, 80 and a miscible diluent liquid selected from the group consisting of xylene, solvent naphtha, chlorbenzene, and nitrobenzene. 85

6. The method of reducing the freezing point of a concentrated anti-knock composition for addition in relatively small proportions to gasoline and like motor fuels, which composition contains, as its principal constituents, tetraethyl lead and an ethylene compound containing halogen atoms at least one of which is a bromine atom, which comprises admixing said composition with an additional miscible diluent liquid having an internal pressure between .90 and 1.08. 95

ROBERT E. WILSON. 100